

## UNITED STATES PATENT OFFICE

EUGENE A. BALSLEY, OF WHEELING, WEST VIRGINIA, AND LUCIEN I. YEOMANS, OF CHICAGO, ILLINOIS, ASSIGNORS TO LUCIEN I. YEOMANS, INC., OF CHICAGO, ILLINOIS, A CORPORATION OF ILLINOIS

## PROCESS OF PROTECTING SAND MOLDS AND CORES

No Drawing.

Application filed July 5, 1929. Serial No. 376,280.

In the preparation of sand molds in which molten metal is to be poured, it is customary to reinforce fragile sections in some instances and to protect corners, small bosses, thin ribs and other projecting surfaces where the wash of the metal is liable to break off or cut away a portion of the mold surface, by using ordinary nails of various sizes which are inserted in the sand body by the molder in such a manner that the nail heads are flush with the mold surface and constitute a part thereof.

On certain classes of work the expense involved in thus protecting the mold from wash is an item of consequence, and it is not uncommon for foundries making irregular sections of large steel castings to use as many as twenty pounds of nails per ton output of the entire foundry, thereby adding a cost of a dollar a ton to the average cost of castings. This is not the only expense, or even the principal expense item occasioned by their use. The proper placing of the nails requires care and skill and involves a considerable labor cost. The expense of shaking out molds after casting is increased, particularly in the case of steel castings as the nail heads are melted by the molten metal and welded to the casting. The labor entailed in chipping off the nails and cleaning the casting is a further item of expense.

We have discovered that the surfaces of a sand mold may be structurally strengthened and protected against wash of molten metal by spraying upon such surfaces a thin layer of molten metal. We may use a variety of metals for this purpose, but have found aluminum well adapted to the requirements, and prefer to use metals which have a marked affinity for oxygen or which upon melting tend to remove rather than increase the gaseous content of the metals from which the casting is to be made. To apply such a coating we prefer to use the well known Schoop spray.

When sprayed upon the mold, the molten metal penetrates into the interstices among

the grains of sand and produces a protective coating which adheres firmly to the mold.

Cores, forming part of a mold, may be treated in this way to expedite cleaning processes after the casting is poured, and structural strength and surface protection against washing may be secured upon dry or green sand cores or upon green or dry sand sections of the mold proper. The roughness of the surfaces of an intricate cored casting may be reduced, as in the case of automobile engine water jackets where resistance to circulation of water is increased by the friction due to rough surfaces and to core material which has been left in the casting because of the difficulty of removing it.

We do not coat the entire surface of the mold or core, but only those surfaces (and particularly fragile projecting portions) which require reinforcement against the wash of the metal. It would be impracticable and even dangerous to coat the entire surface, as the heat of the metal causes vaporization of volatile substances in the mold or core, as, for example, the binder compounds employed in core making. If the entire surface were coated with metal the pressure generated within the core or within the body of the mold, as the case may be, would be liable to cause bursting and distortion and would damage the casting by the formation of blow-holes. With our process the vapors escape from the uncoated surfaces of the mold or core.

The method herein disclosed of protecting sand molds from wash is cheaper than that of inserting nails in the molds, obviates the expense of nails, reduces the cost of cleaning the castings, and in some instances results in a smoother product.

This application is a continuation in part of our application Serial No. 275,956, filed May 7, 1928.

We claim as our invention:

The process of structurally strengthening

the fragile projections and the surfaces adjacent thereto of a sand mold or core to protect such projections from wash which consists in spraying with molten metal such projections and adjacent surfaces, the remaining surface area being not coated with metal in order to permit escape of vapors from such uncoated surfaces.

5 In testimony whereof we have hereunto  
10 affixed our signatures.

EUGENE A. BALSLEY.  
LUCIEN I. YEOMANS.

15

20

25

30

35

40

45

50

55

60

65